# EUROPEAN PATENT SPECIFICATION

(11) **EP 0 128 231 B1**
(45) Date of publication and mention of the grant of the patent: **09.09.1987**
(21) Application number: 83105693.2
(22) Date of filing: 10.06.1983
(51) Int. Cl.: C11D 3/00, C11D 3/30, C11D 1/835, C11D 1/62, D06M 13/46

(54) **Stable concentrated aqueous dispersions of water-insoluble cationic compounds and preparation thereof**
Stabile konzentrierte wässrige Dispersionen von wasserunlöslichen kationischen Verbindungen und deren Zubereitung
Dispersions stables aqueuses concentrées de composés cationiques insolubles dans l'eau et leur préparation

(43) Date of publication of application: 19.12.1984
(73) Proprietor: S.A. Camp Fábrica de Jabones, Granollers Barcelona (ES)
(72) Inventor: Barba, Joaquim M., Barcelona 6 (ES); Cáliz, Joan, Banyoles Girona (ES)
(74) Representative: Klöpsch, Gerald, Dr.-Ing. Patentanwalt

## Description

### Technical field

This present invention deals with concentrated aqueous dispersions or emulsions of insoluble cationic compounds, used as fabric softeners, with an improved stability with time, and in regards to temperature variations in relation to the viscosity and dispersibility in water of the said dispersions. It also deals with the adequate preparation methods for the obtention of the said dispersions.

### State of the former technique

The appearance, in the last years, of more concentrated liquid fabric softener compositions is undoubtedly due to ecnonomical motivations, and to a greater convenience to the consumer. This fact has originated the emergence of serious technical problems related with the increase in active matter, fundamentally insoluble cationic compounds, from concentrations ranging between a 3% to a 7% in the traditional diluted compositions, to proportions higher than 10% in the currently called concentrated softeners. The primary problems have to do with the physical properties of the concentrated compositions, essentially with their viscosity and dispersibility in water and with the variation, in negative sense, of the said properties with temperature and time of storage, as well as with relatively abrupt changes of temperature.

It has been known for a time, for instance in US-Patent No. 3,681,241, that the addition of small quantities of such electrolytes as salts of divalent metals causes a considerable decrease in viscosity. In German Patent No. 29 11 198 there has also been a description of the use of aluminium salts, producing an anti-gelling effect. But these solutions are only partly effective, as the quantity of electrolyte that can possibly be added has to be very small, otherwise there could be problems caused by the formation of clots and rupture of phases. Another attempt to solve this problem consists in substituting soluble cationic products instead of the insoluble cationic products, as described, for instance, in the European Patent Application No. 00 406, but these compositions do not give the required softening performance, as it is necessary for the cationic compound to become bound to the surface of the fabric for the softening effect to occur, and these compounds, because of their solubility in water, are dragged away in a great proportion during the rinsing process. The European Patent Applications Nos. 13 780 and 18 039 describe the use of non-cyclic hydrocarbons, fatty acids or their esters, and fatty alcohols as additives to decrease viscosity and to enhance the stability of concentrated softening compositions, but the effectivity of these compounds decreases noticeably with low storage temperatures, so the solution provided by them is only a partial one. The addition of non-ionic alkoxylated surfactants is known for diluted compositions, and has been applied in concentrated compositions, for instance in the German Patent No. 29 11 198, in the French Patent No. 2 482 636 and in the US-Patent No. 3,947,076, although its utilization has not been sufficiently specified as far as the types of products are concerned, nor as to the effect produced therewith, and, nevertheless, their stabilizing action on viscosity has little effectivity at high temperatures, so it also has to be considered as only a partial answer.

The utilization of alkoxylated amines in softener composition has been known now for some time, as shown in the following documents: US-Patent No. 3,850,818, DE-A-1 19 043, US-Patent No. 4,076,632, US-Patent No. 4,157,307, European Patent Application No. 21 476, US-Patent No. 4,320,013. The part played by the alkoxylated amines in the compositions described by the documents above cited are both of fabric softening and of enhancing the stability of the dispersion, but all of them are referred to diluted softener compositions, and, moreover, the stabilizing action of the alkoxylated amine has to be concurrent with the joint action of other additives, like urea or alcohols. In European Patent Application No. 56 695 is introduced for the first time the concept of the action of alkoxylated amines as factors to achieve a proper viscosity, as well as a satisfactory stability, in concentrated softener compositions, provided that it is asociated to the addition of low levels of electrolyte. Nevertheless, there is a serious limitation, as it is stated that the number of mols of oxyalkyl which conform the two alkoxylated substituents of the amine cannot even be higher than 14 and that preferably it has to be between 2 and 8, as otherwise it should be necessary, to maintain the adequate viscosity, to significantly increase the presence of electrolyte, which would be deleterious to product stability. This limitation reduces the range of what is possible in the technique of obtention of stable concentrated softener compositions, and does not allow the utilization of alkoxylated amines with a high degree of alkoxylation which, moreover, are significantly lower in cost than those of a lower degree of alkoxylation.

### Vindication of the invention

The invention herein solves these problems, as in a surprising way unexpected results are achieved in good characteristics of viscosity and a good dispersibility in water of concentrated aqueous dispersions of insoluble cationic compounds, as well as an extended stabilization thereof in ranges of temperatures between 0° and 50°C, by means of the addition of amines with a high degree of alkoxylation in union with a precise and definite system of two non-ionic components. Also, surprisingly, the dispersions described in the invention herein exhibit an excellent adaptability in the maintenance of their physical properties versus abrupt and wide changes of temperature. Also inherent difficulties to the process of obtention of aqueous concentrated dispersions of cationic softeners are solved.

The fundamental object of the invention herein, then, is to achieve concentrated aqueous dispersions of insoluble cationic softeners with adequate viscosity and dispersibility and an improved stability in storage and in abrupt temperature changes. Another aim of the invention is the achievement of more economically profitable concentrated softener compositions. Another aim of the invention herein is to develop a process to obtain the compositions hereof, easy and dependable in its results.

### Description of the invention

The invention herein relates to fabric softener compositions which are basically constituted by a cationic fabric softener, an alkoxylated amine and nonionic surfactant characterized in that the mixtures contain:
A. from 10% to 20% by weight of a cationic water-in-soluble softener compound, or of a mixture of the such,
B. from 0,1 % to 3% by weight of an alkoxylated tertiary amine, or of its correspondent ammonium salt, having the general formula: wherein R₁ represents an alkyl or alkenyl group between 10 and 20 carbon atoms, n is an integer betwen 1 and 4; x and y represent numbers between 10 and 50, so that the sum thereof is from 20 to 100 (x + y = 20 to 100),
C. 0.5 to 5% by weight preferably 1 to 3% by weight of a mixture of two non-ionic surfactants pertaining to the groups:
   i.-alkoxylated C₈ to C₂₀ fatty alcohols or alkoxylated C₇ to C₁₀ alkyl phenols, with a number of mols of a C₁ to C₄ alkylene oxide from 25 to 75 per mol of alcohol or phenol,
   ii.-alkoxylated C₈ to C₂₀ fatty alcohols or alkoxylated C₇ to C₁₀ alkyl phenols with a number of a C₁ to C₄ alkylene oxide mols from 1 to 5, per mol of alcohol or phenol in such a way that the ratio between i and ii ranges between 10:1 and 1:10,

   the above mentioned compounds being dispersed or dissolved in water with a pH ranging between 3 and 5.

It is highly preferred, in the composition of the invention therein, to add small quantities of an electrolyte, preferably salts of strong acids and divalent metals, the effect of which is very beneficial on the viscosity parameter. The most adequate proportions of the said electrolyte range between 0.02% and 0.15%. Below the inferior limit, the electrolyte action is very unsubstantial, and above the upper limit, there is risk that undesirable phenomena may appear, undermining the stability of the compositions, due to problems of phase disruption.

The insoluble cationic compounds of the invention herein belong to the type usually used in aqueous dispersions with softening activities on textile fabrics, preferably those belonging to the following groups:
1 - Salts of quaternary ammonium with two long chain alk(en)yl groups, C₁₀ to C₂ₒ.
2 - Imidazolinium quaternary salts, with two long chain alk(en)yl groups C₁₀ to C₂ₒ,

and are incorporated into the compositions in a proportion ranging from 10% to 20% by weight of the aforesaid composition, and in a preferred proportion of 11 % to 16% to achieve an optimal ratio of softener activity/viscosity.

The alkoxylated tertiary amines with a number of mols of alkylene oxide of 20 to 100 per mol of amine, are highly important to achieve a viscosity between 50 and 900 mPas with a good stability, during long storage terms. In contradistinction to what was anticipated in the previous technique as expressed in the European Patent No. 56 695, it has been possible to adjust the formula in a surprising way so as to make it feasible that highly alkoxylated amines perform the said function with the presence of small quantities of electrolyte in a range of 500 to 1000 ppm. Notwithstanding the fact that the said amines can be used in proportions ranging from 0.1 % to 3% by weight, the preferred proportions are those from 0.5% to 1.5%, with a view to achieve a good balance between the desired effect of viscosity reduction and the final cost of the composition.

The system of non-ionic surfactants herein shows itself to be effective to achieve compatibility of the alkoxylated amine with a high degree of alkoxylation with the formulation in presence of small amounts of electrolyte, and it is also basic to confer on the dispersion its qualities of elasticity versus temperature changes during storage. These non-ionic surfactants are selected from amongst the group of alkoxylated fatty alcohols or alkoxylated alkylphenols with a general formula: wherein R₂ represents an alk(en)ylic group between C₈ and C₂₀ or phenylalkyl from C, to Cᵢₒ, n is an integer from 1 to 4, and z is a number between 1 and 75.

For a good execution of the invention, it is necessary to use two non-ionic surfactants which are clearly differentiated on their z value:
A) A non-ionic surfactant according to the general formula II, in which z ranges between 25 and 75.
B) A non-ionic surfactant according to the general formula II, in which z ranges between 1 and 5.

Although the proportion between A and B can have a range between 10:1 to 1:10, the preferable proportion is between a range of 3:1 to 1:3.

The process of obtention has also a great importance to obtain good results in viscosity, dispersibility in water, and stability. The temperature during the said process has to be maintained with decreasing rhythm between 60° and 30°C, but the most important factor is the order and rate of addition of the different components. So, for example, it is convenient to add to the water, in the first place, a molten mixture of the alkoxylated amine together with the system of non-ionic surfactants, and to adjust the pH by means of a strong acid between 3 and 5. The addition of the insoluble cationic compound is performed in a fractionated way, alternating with additions, also in a fractioned way, of the electrolyte. Small variations in the order of addition are the cause of dispersions with a very high initial viscosity or with a bad performance versus temperature variations.

The characteristics of the dispersions so obtained are in general as follows:
- pH = 3 to 5
- Specific Gravity = 0.95 to 1.05 g/cc
- Initial Viscosity - 50 to 400 mPas
- Viscosity after 8 weeks at room temperature = 50 to 400 mPas
- Viscosity after 2 weeks at 0°C to 5°C: Less than 900 mPas
- Viscosity after 2 weeks at 45°C: Less than 900 mPas
- Dispersibility in water: Excellent,

these characteristics being very appropriate from the viewpoint of its storage and of its use as a fabric liquid softener composition.

The detailed description of the different components of the invention herein are described below.

The insoluble cationic compounds are the active softening matter, and can be selected from amongst the following groups:
1. Quaternary acyclic ammonium salts represented by the general formula: wherein R₃ and R₄ represent alkyl or alkenyl groups of from 10 to 20 carbon atoms, R₅ and R₆ represent short alkyl groups from 1 to 4 carbon atoms, and A- represents the salt counteranion of a strong acid, as, for example, halides or methyl sulphate. These are very widely known products and, as examples, the following could be quoted: ditallow dimethyl ammonium chloride; dicoco dimethyl ammonium chloride; distearyl dimethyl ammonium chloride; di(hydrogenated-tallow) dimethyl ammonium methyl sulfate; di(hydrogenated tallow) dimethyl ammonium chloride; ditallow dimethyl ammonium methyl sulfate. They are easily available in the market under different trademarks, like Adogen®, Varisoft® (Sherex Chemicals), Quartamin@ (Kao Corp.), Arquad® (Akzo), Präpagen® (Hoechst, etc.... Of these, di(hydrogenated tallow) dimethyl ammonium chloride is preferred.
2. Quaternary imidazolinium salts represented by the general formulae: where R₇, Rₛ, Rg and R₁₀ represent saturated or unsaturated alkyl groups, with 10 to 20 carbon atoms, and A- represents the salt counteranion of a monoprotic acid, such as, for example, halide or methyl sulfate. This type of products is also well known, and as examples the following are quoted:

Methyl-1-(hydrogenated tallow) amido ethyl-2-(hydrogenated tallow) imidazolinium methyl sulfate; methyl-1-tallow amido ethyl-2 tallow imidazolinium methyl sulfate; methyl-l-oleyl amido ethyl-2-oleyl imidazolinium chloride; 1-ethylene bis(2-tallow, 1-methyl imidazolinium methyl sulfate). Preferred compounds are methyl-1-(hydrogenated tallow) amido-ethyl-2-(hydrogenated tallow) imidazolinium methyl sulfate, marketed by Sherex Chemical Company under the designation Varisoft® 445, and 3-methylethyl-1-(hydrogenated tallow) amido ethyl-2-(hydrogenated tallow) imidazolinium methyl sulfate, marketed by Rewo Chemische under the designation Rewoquat^{e} W7500H.

The alkoxylated amines have the general formula I, wherein R₁ represents an alkyl or alkenyl group having from 10 to 20 carbon atoms, those corresponding to coconut, oleic, tallow, hydrogenated tallow, and hydrogenated tallow being preferred; n is an integer from 1 to 4, value 2 being preferred, which corresponds to ethoxylated amines. The values of x and y range between 10 and 50 in such a way that the total sum thereof ranges from 20 to 100, this is to say, the number of mols of ethylene oxide per amine mol must range from 20 to 100, although the preferred values of x + y range from 20 to 50. This type of products is available in the market under various commercial designations as, for example, Etilenox® (Pulcra), Ethomeen® (Akzo), Genamin@ (Hoechst). Highly preferred are the amines of hydrogenated tallow with 20 mols of ethylene oxide such as Etilenox® KM-30 of Pulcra, S.A. and Genamin® S-250 of Hoechst A.G., and with 50 mols of ethylene oxide as, for example, Ethomeen® HT60 of AKZO Chemie.

Non-ionic surfactants have the general formula II, wherein R₂ represents an alkyl group of from 8 to 20 carbon atoms, for example, those corresponding to fatty alcohols like lauric, myristic, palmitic or stearic alchols, or the mixtures thereof, or an alkyl phenyl group with 7 to 10 carbons, as those corresponding to the alkyl phenols with 8 and 9 carbon atoms. The preferred groups are those corresponding to the lauric alcohol and nonylphenol. The value of n can be from 1 to 4, being the preferred value that of 2, and, therefore, the ethoxylated products. According to the invention herein, a binary system of non-ionic oxyethylenated surfactants is necessary in function of the Z value:
A) A non-ionic surfactant according to general formula II and with a Z value between 25 and 75, the preferred values being between 25 and 50.
B) A non-ionic surfactant according to the general formula II with a Z value between 1 and 5, preferably between 1 and 3.

in a weight ratio in the range from 10:1 to 1:10, the preferred weight ratio being that of between 3:1 and 1:3. These products are well available in the market and can be found under the following commercial designations: Dobanol® (ICI), Dowfax@ (Dow Chemical), Emulgen@ (Kao Corp.), Catinex® (Pulcra, S.A.), etc..

.. Especially preferred is the binary system nonylphenol with 30 mols of ethylene oxide together with nonylphenol with 1.5 moles of ethylene oxide, with a weight ratio ranging from 3:1 to 1:3.

Besides the essential components, a series of optional additives can be incorporated to the compositions of the invention herein which are conventionally used in the field of fabric softeners, like dyes, perfumes, supplementary viscosity modifiers, emulgents, optical brighteners, antioxidants, germicides, fungicides, moisteners, etc....

It is especially indicated, for a better viscosity control, the use of electrolytes, as salts of divalent metals with strong acids, in weight ratios ranging between 200 and 1,500 ppm. Especially preferred electrolytes are calcium chloride and magnesium sulfate.

Other optional additives, which are indicated as auxiliary in viscosity control, are linear or branched short chain alcohols from 1 to 4 carbon atoms. Isopropyl alcohols, particularly, may be present in a proportion between 1 % and 4%, but not in a bigger proportion that may cause lack of stability.

Optional components indicated to improve the water absorbancy of the fabrics treated with the softeners are the emulsified silicones, such as DC-347, DC-346 and DC-HV490, marketed by Dow Corning. Small amounts, of an order of 0.01% to 0.3% in active matter, are employed.

Optical brighteners can also be employed, like, for example, derivatives of stilbene and distyrylbiphenyl, marketed by Ciba-Geigy as Tinopal®.

It is convenient here to remark that, in what concerns the more detailed aspects of the process of obtention given by the invention herein, that the said process exhibits two very distinct phases:
A- The addition of a molten mixture of the non-ionic components and the alkoxylated amine to water, with stirring, at a temperature between 50° and 60°C, and the addition of a strong acid up to a pH between 3 and 5.

B - Addition of the molten cationic component in two fractions, of preferably 70% and 30%, respectively, of the total amount, alternating with the addition of electrolyte, also in two fractions corresponding to 30% and a 70% of the total quantity of the same, in such a way that after the first addition of the 70% of the cationic compound follows the 30% of the electrolyte, and that, following a time of stirring and mixing, the second fraction of a 30% of the cationic component is added and, upon this, the remaining 70% of electrolyte. All this part of the process takes place with stirring and at a temperature between 45° and 55°C.

Once the dispersion has taken place in the manner hereinabove, it is left to cool to 30° to 40°C, adjusting the pH again between 3 and 5, and the remaining optional ingredients can now be added.

It is important to remark that the order of addition hereinbefore is essential to achieve dispersions with the desired viscosity and stability.

For a better understanding of the description of the invention given herein, the following examples are given, with the statement that they must not be construed as restrictions to the aforesaid invention:

### Example I

1.5 parts of ethoxylated hydrogenated tallow amine with 25 mols of ethylene oxide per mol of amine are mixed, at a temperature of 55°C, together with 1 part of ethoxylated nonylphenol with 30 mols of ethylene oxide per mol of nonylphenol and 1 part of ethoxylated nonylphenol with 1.5 mols of ethylene oxide per mol of nonylphenol. The said molten mixture is added to 70 parts of deionized water, at a temperature of 50° to 60°C, and with strong stirring. Hydrochloric acid 1 N is added until a pH of 3 to 4 is reached. Upon this, and keeping a temperature between 50° and 55°C, and a strong stirring, 11.7 parts of molten di(hydrogenated tallow) dimethyl ammonium chloride are added, with an active matter content of a 75%, and after this 0.03 parts of calcium chloride are added, in 10% aqueous solution. The mixture is stirred for 5 minutes, and then 5.0 more parts of molten cationic component are added and 0.07 parts of calcium chloride. The dispersion is cooled to 40°C in 10 minutes, maintaining the stirring on, and 0.6 parts of DC-HV490 are added (a 35% silicone emulsion marketed by Dow Corning). It is left to cool to 30° to 35°C, and other optional ingredients are added, as desired, such as perfume, dyes, etc... and deionized water is added to make up 100 parts. The dispersion is cooled to 25°C, and pH is brought to between 3.5 and 4.5 and, after this, the product is bottled.

With the dispersion prepared as hereinbefore, the following tests and measurements are performed:
Initial Viscosity. - The dispersion is left to settle until the day following its preparation, and its viscosity is measured at 20°C with a Brookfield LV Viscosimeter. Initial viscosity for the solution thus prepared is 200 mPas.

Stability at room temparature. - The dispersion, well packed and closed, is stored at a temperature of 25°C±5°C for two months, and at the end of this period a viscosity measurement is performed at 20°C. The viscosity value observed for the dispersion thus prepared is 210 mPas.

Stability at high temperatures. - A sufficient amount of sample of the dispersion is hermetically sealed in the same vessel where the viscosity value is to be determined, and it is kept in a stove at 45°C during five days. Then, the sample is removed from the stove, left for another day at room temperature, and its viscosity is measured at 20°C. The sample is again hermetically sealed and it is again placed in the stove at 45°C, and it is again removed at the end of that period, it is left to stabilize during another day at room temperature and its viscosity is measured at 20°C. The values that have been found are:
Viscosity after 5 days = 380 mPas
Viscosity after 10 days = 850 mPas

Stability at low temperatures. - A sample of the dispersion is hermetically sealed in the same vessel where the viscosity is to be tested, and it is placed in a refrigerator at 3°C±2°C. The sample is removed after five days, it is left for another day at room temperature and its viscosity is tested at 20°C.

The sample is again placed in the refrigerator, for another four days, and then it is removed, left to stabilize for one day at room temperature, and then the viscosity is tested at 20°C. The values of viscosity that have been found are:
Viscosity at 5 days = 425 mPas
Viscosity at 10 days = 800 mPas

Elasticity versus temperature. - Sample of the dispersion is taken, and placed in an appropriate vessel, it is placed in a bath provided with a temperature regulator, and the temperature is adjusted at 20°C and the viscosity is then measured. It is heated to 70°C in 30 minutes, and the viscosity is again measured. It is cooled again to 20°C in 30 minutes, and the viscosity is tested. The values found are:
Viscosity at 20°C = 200 mPas
Viscosity at 70°C = 490 mPas
Viscosity at 20°C = 325 mPas

Dispersibility in water. ―This test is approximate and orientative. A graduate cylinder is filled with a liter of water at 20°C±5°C of temperature, and with a hardness of 20°FH. 30 grams of the dispersion, which has been kept two months stored at a temperature of 20°C±5°C, are poured on the surface from a height of 8 cm. That part of the dispersion which results not dispersed in the water remains in a ring shape in the higher or lower part of the graduated cylinder, according to its density, and an arbitrary scale is assigned to it, from 0 to 10. 0 means total dispersion and 10 no dispersion. The volume of water to which the dispersion has not arrived is measured, so that the optimal volume is that of 0 ml, and the worst one is that of 1000 ml.

By means of these data, an approximated and arbitrary scale is made, as follows:

Applying these criteria to the dispersion obtained by the invention herein, its dispersibility in water is excellent.

### Example II

Performing the same operations as described under example I, a dispersion is prepared with the following ingredients:

The dispersion exhibits the following characteristics, determined according to the criteria established in example I:

### Example III

Performing the same operations as described herein under example I, a dispersion is prepared with the following ingredients:

The dispersion value exhibits the following characteristics, determined according to the criteria established in example I:

### Example IV

Performing the same operation as described herein under example I, a dispersion is prepared with the following ingredients:

The dispersion exhibits the following characteristics, determined according to the criteria established in example I:

The dispersions described in the examples I to IV exhibit excellent viscosity, dispersibility and stability characteristics during storage and in extreme temperature conditions for their use as fabric concentrated softeners.

### Examples V to XIV

It is the purpose in the following examples to show the importance of the amine with a high degree of alkoxylation, and of the system of non-ionic surfactants in the viscosity, dispersibility in water, and stability of the dispersions. To the end of the establishment of comparative criteria, some basic aspects, such as the contents in active insoluble cationic matter, nature and contents of the alkoxylated amine, and total contents in non-ionic surfactant, have been harmonized.

The abbreviation to design the different ingredients are as follows:
DHTDMAC: Di(halogenated tallow) dimethyl ammonium chloride
DTIMS-3M: 3-methyl-1-tallow amido ethyl-2 tallow imidazolinium methyl sulfate
HTA 25: Hydrogenated tallow amine with 25 mols of Ethylene oxide
NP 30: Nonyl phenol with 30 mols of Ethylene oxide
NP 14: Nonyl phenol with 14 mols of Ethylene oxide
NP 9: Nonyl phenol with 9 mols of Ethylene oxide
NP 1,5: Nonyl phenol with 1.5 mols of Ethylene oxide
LA 50: Lauric alcohol with 50 mols of Ethylene oxide
LA 2,7: Lauric alcohol with 2.7 mols of Ethylene oxide
Tween@ 60: Polyoxyethylene sorbitane monostearate (ICI)
GLYC (OP-OE): Glycerine with 8 mols of Ethylene oxide and 28 mols of propylene oxide
Plurafac^{@} 40: Polyalkoxylated alcohol, from 13 to 15 carbon atoms, marketed by Ugine Kuhlmann.

In Table 1 are shown the different compositions prepared following the basic ideas as described in example I, and in Table 2 their characteristics are detailed according to the criteria given in example I.

On checking the data in Tables 1 and 2, it can be inferred that the addition of the highly alkoxylated amine causes an improvement in the stability of the compositions at room temperature and an improvement in the dispersibility of the compositions in water. The incorporation of non-ionics improves the stability at low temperatures, but it is not effective at high temperatures. All dispersions with a system of non-ionics as described in the invention herein cause an improvement of stability both at low and at high temperatures, and cause the viscosity value at room temperature to stay practically unchangeable, and give an excellent dispersibility in water.

## Claims

1. Fabric concentrated softener compositions with good viscosity and dispersibility in water and an improved stability versus a long period of storage, and versus temperature changes, its essential components being a cationic fabric softener, an alkoxylated amine, and non-ionic surfactants characterized in that the compositions contain:
A. 10 to 20% by weight of a water-insoluble cationic fabric softener compound, or a mixture of thereof,
B. 0,1 to 3% by weight of a tertiary alkoxylated amine or its corresponding ammonium salt, with a general formula as follows: wherein R₁ represents an alkyl or alkenyl group with 10 and 20 carbon atoms, n is an integer from 1 to 4, and x and y represent numbers between 10 and 50, the sum of both being from 20 to 100 (x + y = 20 to 100).
C. 0.5 to 5% by weight of a mixture of two non-ionic surfactants belonging to the following groups:
i.-alkoxylated C₈ to C₂₀ fatty alcohols or alkoxylated C₇ to C₁₀ alkyl phenols, with a number of mols of a C₁ to C₄ alkylene oxide per mol of alcohol or phenol ranging from 25 to 75,
ii.-alkoxylated C₈ to C₂₀ fatty alcohols or alkoxylated C₇ to C₁₀ alkyl phenols with a number of mols of a C₁ to C₄ alkylene oxide ranging from 1 to 5, in such a way that the weight proportion of the said mixture of non-ionic surfactants is in the range from 10:1 and 1:10,
the said ingredients being dissolved or dispersed in water at a pH ranging between 3 and 5.

2. Compositions according to claim 1 characterised in that the water-insoluble cationic component or components are selected from amongst the following groups:
A. Non-cyclical quaternary ammonium salts having the general formula wherein R₃ and R₄ represent C₁₀ to C₂₀ alkyl or alkenyl groups, R₅ and R₆ represent short chain C₁ to C₄ alkyl groups and A- represents the salt counteranion from a strong acid.
B. Quaternary imidazolinium salts having the following general formulae: wherein R₇, Rₒ, Rg and R₁₀ represent saturated or unsaturated alkyl groups, with chains from 10 to 20 carbon atoms, and A- represents the counteranion of a strong acid.

3. Compositions according to claims 1 and 2, wherein the water-insoluble cationic component or components are: Di(hydrogenated tallow) dimethyl ammonium chloride and/or 3-methyl-1-(hydrogenated tallow) amido ethyl-2-(hydrogenated tallow) imidazolinium methyl sulfate.

4. Compositions according to claims 1 to 3, characterized in that the tertiary alkoxylated amine is: Ethoxylated (hydrogenated tallow) amine with 25 mols of ethylene oxide or ethoxylated (hydrogenated tallow) amine with 50 mols of ethylene oxide.

5. Compositions according to claims 1 to 4, characterized in that the highly alkoxylated non-ionic surfactant component is selected from amongst ethoxylated nonyl phenol with 30 mols of ethylene oxide or ethoxylated lauric alcohol with 50 mols of ethylene oxide and the non-ionic surfactant with a low level of alkoxylation is selected from amongst ethoxylated nonyl phenol with 1.5 mols of ethylene oxide or ethoxylated lauric alcohol with 2.7 mols of ethylene oxide.

6. Compositions according to any preceding claim, characterized in that an electrolyte is added to them as an agent to improve the value of viscosity, belonging to the salts of divalent metals with strong acids, with a weight ratio ranging between 0.02% and 0.15% of the total weight of the composition.

7. Compositions according to any preceding claim, characterized by having the following components:
A. 11 to 16% by weight of a water-insoluble cationic softener compound or a mixture thereof,
B. 0.5 to 1.5% by weight of an alkoxylated tertiary amine having the general formula I, with 20 to 100 mols of alkylene oxide per mol of amine,
C. 1 to 3% by weight of a mixture of two non-ionic surfactants pertaining to the following groups:
i.-alkoxylated C₈ to C₂₀ fatty alcohols or alkoxylated C₇ to C₁₀ alkyl phenols with a number of mols of a C₁ to C₄ alkylene oxide ranging from 25 to 75 per mol of alcohol or phenol
ii.-alkoxylated C₈ to C₂₀ fatty alcohols or alkoxylated C₇ to C₁₀ alkyl phenols with a number of a C₁ to C₄ alkylene oxide mols ranging from 1 to 5 per mol of alcohol or phenol
wherein the weight ratio between the two non-ionic surfactants is in the range from 3:1 to 1:3.
D. 0.03 to 0.15% by weight of an electrolyte, belonging to the said type of salts of divalent metals with strong acids,
the said ingredients being dissolved or dispersed in water at a pH ranging between 3.5 and 4.5.

8. A method of making the compositions according to any preceding claim, characterized in that in a first stage a molten mixture of the non-ionic components is added with stirring together with the alkoxylated amine to deionized water at a temperature between 50°and 60°C and the addition of a strong acid up to a pH between 3 and 5, in a second stage a fractioned addition of the water-insoluble cationic compound is effected, alternating with fractioned additions of electrolyte, all this with stirring and at a temperature between 45° and 55°C, and the preparation of the composition being finished after cooling from 30° to 40°C and adjusting the pH to from 3 to 5, with the addition of optional ingredients.

9. A method according to claim 8, characterized by the addition of the water-insoluble cationic compound in two fractions, the first of them being of a 70% of the total amount and the second to the 30% of the said total amount, alternating with the addition of the electrolyte also in two fractions, the first being of a 30% of the total amount, and the second of a 70% of the total amount.

## Patentansprüche

1. Konzentrierte Weichspülerzusammensetzungen mit guter Viskosität und Dispergierbarkeit in Wasser und verbesserter Stabilität über lange Lagerdauer und gegen Temperaturschwankungen, deren wichtige Bestandteile ein kationischer Weichspüler, ein alkoxyliertes Amid und nichtionische, oberflächenaktive Substanzen bilden, dadurch gekennzeichnet, daß die Zusammensetzungen enhalten:
A. 10 bis 20 Gew.-% einer wasserunlöslichen, kationischen Verbindung mit weichmachender Wirkung für Gewebe oder einer Mischung solcher Verbindungen,
B. 0,1 bis 3 Gew.% eines tertiären Amids oder dessen Ammoniumsalzes der allgemeinen Formel: worin R₁ eine Alkyl- oder Alkenylgruppe mit 10 bis 20 Kohlenstoffatomen ist, n eine ganze Zahl von 1 bis 4 ist und x und y Zahlen zwischen 10 und 50 darstellen, deren Summe 20 bis 100 beträgt (x + y = 20 bis 100).
C. 0,5 b is 5 Gew.-% einer Mischung aus zwei nichtionischen, oberflächenaktiven Substanzen, die zu folgenden Gruppen gehören:
1.-alkoxylierte C₈- bis C2o-Fettalkohole oder alkoxylierte C₇- bis Cₗₒ-Alkylphenole mit einer Molanzahl eines Cᵢ- bis C₄-Alkylenoxids von 25 bis 75 pro Mol Alkohol oder Phenol,
ii.-alkoxylierte C₈- bis C₂₀-Fettalkohole oder alkoxylierte C₇- bis C₁₀-Alkylphenole mit einer Molanzahl eines C₁- bis C₄-Alkylenoxids von 1 bis 5,
so daß das Gewichtsverhältnis dieser Mischung aus nichtionischen, oberflächenaktiven Substanzen zwischen 10:1 und 1:10 liegt,
wobei die genannten Bestandteile in Wasser bei einem pH-Wert zwischen 3 und 5 gelöst oder dispergiert werden.

2. Zussamensetzungen nach Anspruch 1, dadurch gekennzeichnet, daß der wasserunlösliche, kationische Bestandteil oder die wasserunlöslichen, kationischen Bestandteile aus einer der folgenden Gruppen ausgewählt sind:
A. Nichtzyklische, quaternäre Ammoniumsalze der allgemeinen Formel: worin R₃ und R₄ C₁₀- bis C₂₀-Alkyl- oder -Alkenylgruppen, R₅ und R₆ kurzkettige C₁- bis C₄-Alkenylgruppen sind, und A- das Anion einer starken Säure darstellt,
B. quaternäre Imidazoliniumsalze de allgemeinen Formeln: worin R₇, R₈, Rg und R₁₀ gesättigte ode ungesättigte Alkylgruppen mit Ketten von 10 bis 20 Kohlenstoffatomen sind und A- das Anion einer starken Säure ist.

3. Zusammensetzungen nach einem der Ansprüche 1 und 2, dadurch gekennzeichnet, daß der wasserunlösliche, kationische Bestandteile oder die wasserunlöslichen, kationischen Bestandteile Di(hydrierter Talg) dimethylammoniumchlorid und/oder 3-Methyl-1-(hydrierter Talg) amidoethyl-2-(hydrierter Talg) imidazolmethylsulfat ist/sind.

4. Zusammensetzungen nach einem der Ansprüche 1 bis 3, dadurch gekennzeichnet, daß das tertiäre alkoxylierte Amin ethoxyliertes (hydrierter Talg) Amin mit 25 Molen Ethylenoxid oder ethoxyliertes (hydrierter Talg) Amin mit 50 Molen Ethylenoxid ist.

5. Zusammensetzungen nach einem der Ansprüche 1 bis 4, dadurch gekennzeichnet, daß der Bestandteil der hoch alkoxylierten nichtionischen oberflächenaktiven Substanz aus der Gruppe aus ethoxyliertem Nonylphenol mit 30 Molen Ethylenoxid oder ethoxyliertem Laurinalkohol mit 50 Molen Ethylenoxid ausgewählt wird und die nichtionische oberflächenaktive Substanz mit geringer Alkoxylierung aus der Gruppe aus ethoxyliertem Nonylphenol mit 1,5 Molen Ethylenoxid oder ethoxyliertem Laurinalkohol mit 2,7 Molen Ethylenoxid ausgewählt wird.

6. Zusammensetzungen nach einem der vorangeganenen Ansprüche, dadurch gekennzeichnet, daß ein Elektrolyt, welcher zu den Salzen der zweiwertigen Metalle mit starken Säuren gehört, als Mittel zur Verbesserung des Viskositätswerts in einem Gewichtsverhältnis von 0,02% bis 0,15%, bezogen auf das Gesamtgewicht der Zusammensetzung, zugegeben wird.

7. Zusammensetzungen nach einem der vorangegangenen Ansprüche, dadurch gekennzeichnet, daß sie die folgenden Bestandteile aufweisen:
A. 11 bis 16 Gew.-% eines wasserunlöslichen, kationischen Weichmachers oder einer Mischung solcher Weichmacher
B. 0,5 bis 1,5 Gew.-% eines alkoxylierten, tertiären Amins der allgemeinen Formel I mit 20 bis 100 Molen Alkylenoxid pro Mol Amin,
C. 1 bis 3, Gew.-% einer Mischung aus zwei nichtionischen, oberflächenaktiven Substanzen, die zu den folgenden Gruppen gehören:
i.-alkoxylierte C₈- bis C₂₀-Fettalkohole oder alkoxylierte C,- bis C₁₀-Alkylphenole mit einer Molanzahl eines Cᵢ- bis C₄-Alkylenoxids von 25 bis 75 pro Mol Alkohol oder Phenol,
ii.-alkoxylierte Cₐ- bis C₂₀-Fettalkohole oder alkoxylierte C₇- bis C₁₀-Alkylphenole mit einer Anzahl an C₁- bis C₄-Alkylenoxidmolen von 1 bis 5 pro Mol Alkohol oder Phenol,
wobei das Gewichtsverhältnis der beiden nichtionischen, oberflächenaktiven Substanzen zwischen 3:1 und 1:3 liegt,
D. 0,03 bis 0,15 Gew.-% eines Elektrolyten, welcher zu den Salzen der zweiwertigen Metalle mit starken Säuren gehört,
wobei die genannten Bestandteile in Wasser bei einem pH-Wert zwischen 3,5 und 4,5 gelöst oder dispergiert werden.

8. Verfahren zur Herstellung der Zusammensetzungen nach einem der vorangeganenen Ansprüche, dadurch gekennzeichnet, daß in einem ersten Schritt eine flüssige Mischung aus nichtionischen Bestandteilen und dem alkoxylierten Amin unter Rühren zu entionisiertem Wasser bei einer Temperatur zwsichen 50°C und 60°C sowie eine starke Säure mit einem pH-Wert zwischen 3 und 5 zugegeben wird, und in einem zweiten Schritt eine fraktionierte Zugabe des wasserunlöslichen kationischen Bestandteils im Wechsel mit fraktionierten Zugaben des Elektrolyten unter Rühren bei einer Temperatur zwischen 45°C und 55°C erfolgt, wobei die Herstellung de Verbindung nach Abkühlen auf 30°C bis 40°C und Einstellen des pH-Werts auf 3 bis 5 unter Zugabe der wahlweisen Bestandteile beendet wird.

9. Verfahren nach Anspruch 8, gekennzeichnet durch die Zugabe der wasserunlöslichen, kationischen Verbindung in zwei Fraktionen, wobei die erste 70% des Gesamtanteils und die zweite 30% des Gesamtanteils ausmacht, im Wechsel mit der Zugabe des Elektrolyten ebenfalls in zwei Fraktionen, wobei die erste 30% des Gesamtanteils und die zweite 70% des Gesamtanteils ausmacht.

## Revendications

1. Compositions concentrées d'adoucissants pour tissus avec une viscosité adéquate, bien dispersibles dans l'eau et avec une stabilité améliorée pendant de longues durées de stockage et vis-à-vis des changements de la température, dont les constituants essentiels sont un adoucissant cationique pour les tissus, une amine alcoxylée et des agents tensio-actifs non ioniques, caractérisées en ce qu'elles contiennent:
A. 10 à 20% en poids d'un agent adoucissant les tissus cationique insoluble dans l'eau ou d'un mélange de tels agents:
B. 0,1 à 3% en poids d'une amine tertiaire alcoxylée ou d'un sel d'ammonium d'une telle amine, de la formule générale dans laquelle R₁ désigne un radical alkyle ou alcényle en C₁₀ à C₂₀, n est un nombre entier valant de 1 à 4 et x et y sont des nombres compris entre 10 et 50 de telle façon que la somme x + y = 20 à 100;
C. 0,5 à 5% en poids d'un mélange de deux agents tensio-actifs non ioniques choisis parmi les groupes ci-après:
i.―les alcools gras en Cₐ à C₂₀ alcoxylés et les alkyl-phénols en C₇ à C₁₀ alcoxylés avec 25 à 75 moles d'un oxyde d'alkylène en Ci à C₄ par mole d'alcool ou de phénol;
ii.―les alcools gras en Cₛ à C₂₀ alcoxylés et les alkyl-phénols en C₇ à C₁₀ alcoxylés avec 1 à 5 moles d'un oxyde d'alkylène (lire: par mole d'alcool ou de phénol),
de façon telle que la proportion pondérale de ce mélange d'agents tensio-actifs non ioniques soit comprise (lire: que le rapport pondéral entre les deux agents tensio-actifs de ce mélange soit compris) dans la gamme de 10:1 à 1:10,
ces ingrédients étant dissous ou dispersés dans de l'eau à un pH allant de 3 à 5.

2. Compositions suivant la revendication 1, caractérisées en ce que le ou les agents cationiques insoluble(s) dans l'eau est (sont) choisi(s) dans les groupes ci-après
A. les sels d'ammonium quaternaire non cycliques de la formule générale dans laquelle R₃ et R₄ désignent chacun un radical alkyle ou alcényle en C₁₀ à C₂₀ et R₅ et R₆ désignent chacun un radical alkyle à courte chaîne en C₁ à C₄, tandis que A- représente le contre-anion du sel d'un acide fort;
B. les sels d'imidazolinium quaternaires de l'une des formules générales ci-après: dans lesquelles R₇, R₈, Rg et R₁₀ désignent des groupes alkyle saturés ou non saturés avec des chaînes en C₁₀ à C₂₀ et A- représente le contre-anion d'un acide fort.

3. Compositions suivant les revendications 1 et 2, caractérisées en ce que le composant cationique insoluble dans l'eau est le chlorure de di(suif hydrogéné)-diméthyl-ammonium et(ou) le méthyl-sulfate de 3-méthyl-1-(suif hydrogéné)amido-éthyl-2-(suif hydrogéne)-imidazolinium.

4. Compositions suivant les revendications 1 à 3, caractérisées en ce que l'amine tertiaire alcoxylée est une amine de suif hydrogène éthoxylée par 25 ou 50 moles d'oxyde d'éthylène.

5. Compositions suivant les revendications 1 à 4, caractérisées en ce que l'agent tensio-actif non ionique fortement alcoxylé est choisi parmi le nonylphénol éthoxylé par 30 moles d'oxydes d'éthylène et l'alcool laurylique éthoxylé par 50 moles d'oxyde d'éthylène, tandis que l'agent tensio-actif non ionique à faible taux d'alcoxylation est du nonyl-phénol éthodylé par 1,5 mole d'oxyde d'éthylène ou de l'alcool laurylique éthoxylé par 2,7 moles d'oxyde d'éthylène.

6. Compositions suivant l'une quelconque des revendications précédentes, caractérisées en ce qu'elles contiennent en outre, en tant qu'ingrédient destiné à améliorer leur viscosité, en électrolyte choisi parmi les sels d'acides forts de métaux bivalents, et ce en une proportion comprise entre 0,02 et 0,15% de leur poids total.

7. Compositions suivant l'une quelconques des revendications précédentes, caractérisées en ce qu'elles comprennent les constituants ci-après:
A. 11 à 16% d'un agent adoucissant cationique insoluble dans l'eau ou d'un mélange de tels agents;
B. 0,5 à 1,5% en poids d'une amine tertiaire alcoxylée de la formule générale I avec 20 à 100 moles d'un oxyde d'alkylène par mole d'amine;
C. 1 à 3% en poids d'un mélange de deux agents tensio-actifs non ioniques choisis parmi
i.-les alcools gras en C₈ à C₂₀ alcoxylés et les alkyl-phénols en C₇ à C₁₀ alcoxylés avec 25 à 75 moles d'un oxyde d'alkylène en C₁ à C₄ par mole d'alcool ou de phénol, et
ii.-les alcools gras en C₈ à C₂₀ alcoxylés et les alkyl-phénols en C₇ à C₁₀ alcoxylés avec 1 à 5 moles d'un oxyde d'alkylène par mole d'alcool ou de phénol;
le rapport pondéral entre les deux agents tensio-actifs étant compris entre 3:1 et 1:3;
D. 0,03 à 0,15% en poids d'un électrolyte choisi parmi les sels d'acides forts d'un métal bivalent, ces composants étant dissous ou dispersés dans de l'eau à un pH compris entre 3,5 et 4,5.

8. Procédé de préparation d'une composition suivant l'une des revendications précédentes, caractérisé en ce que, dans le premier stade, l'on ajoute sous agitation le mélange fondu des composants non ioniques et l'amine alcoxylée à de l'eau désionisée, à une température comprise entre 50 et 60°C, le pH étant ajusté à l'aide d'un acide fort entre 3 et 5, puis l'on ajoute alternativement, dans un deuxième stade, entre 45 et 55°C et sous agitation continue, des portions de l'ingrédient cationique insoluble dans l'eau et des portions de l'électrolyte, on refroidit le mélange entre 30 et 40°C et on complète la préparation de la composition par l'ajustement de son pH entre 3 et 5 et l'addition d'autres ingrédients éventuels.

9. Procédé suivant la revendication 8, caractérisé en ce que l'addition du composé cationique insoluble dans l'eau est réalisée en deux étapes, l'addition de 70% de ce composé étant suivie de celle de 30% de la quantité totale de l'électrolyte et l'addition finale des 30% restants de celles des 70% restants de l'électrolyte.
